

## UNITED STATES PATENT OFFICE.

EMILE BINDSCHEDLER, OF PHILADELPHIA, PENNSYLVANIA, AND GEORGE JUER, OF HOPEWELL, VIRGINIA, ASSIGNORS TO TUBIZE ARTIFICIAL SILK COMPANY OF AMERICA, OF WILMINGTON, DELAWARE, A CORPORATION OF DELAWARE.

PROCESS OF MANUFACTURING ARTIFICIAL SILK AND OTHER PRODUCTS FROM NITROCELLULOSE.

No Drawing.

Application filed November 19, 1920. Serial No. 425,049.

To all whom it may concern:

Be it known that we, EMILE BINDSCHEDLER, a citizen of the Republic of Switzerland, and resident of Philadelphia, in the 5 county of Philadelphia, in the State of Pennsylvania, and GEORGE JUER, recently a subject of the former Austro-Hungarian Empire, and now a resident of Hopewell, in the county of Prince George, in the State 10 of Virginia, have invented certain new and useful Improvements in Processes of Manufacturing Artificial Silk and Other Products from Nitrocellulose, of which the following is a true and exact description.

15 Our invention relates to the manufacture of articles from nitrocellulose and particularly to the production of artificial silk. Heretofore it has been known that acetone and its homologues are solvents of nitrocellulose and that its or their use as such would be advantageous from the point of view of the comparatively easy and large percentage of their recovery as compared with other solvents the large losses of which 20 more than offset their relative cheapness. It has been found, however, that acetone as heretofore attempted to be used, resulted in a cloudiness or opacity in the finished product made from the acetone collodion 25 and, particularly, it is found that artificial silk so made is friable and without lustre.

The object of our invention is to provide a method of using acetone as a solvent for nitrocellulose and for recovering the nitrocellulose from solution after manufacture 35 which will produce a lustrous and strong filament or other product and we accomplish this by dissolving nitrocellulose in a solvent consisting in whole or in part of acetone or its homologues by imparting to 40 the acetone collodion thus produced the desired form in the case of artificial silk, forming it into a fine filament by forcing it through spinnarettes and by extracting the 45 solvent from the formed product by immersing said product in a liquid or solution which is mixable with acetone and in which nitrocellulose is insoluble. This extraction of the solvents can be effected by 50 immersing the spools or bobbins on which the fibres are wound in a bath of such a liquid or by providing a coagulating bath through which the fibres pass.

By preference we first dehydrate the nitrocellulose before dissolving it which can 55 be well effected by treating it with ethyl-alcohol which need not be extracted before the acetone solvent is applied to the nitrocellulose and by preference also we use dry acetone as a solvent as described in our co-pending application filed November 19, 1920, Serial No. 425,048, which is intended 60 to cover the method involving the dehydration of the nitrocellulose and the use of dry acetone as a solvent. Our present invention 65 having to do with the particular method of extracting the solvent from the filament or other product made from the acetone collodion which involves the use of the liquid mixable with acetone and without effect upon the nitrocellulose, irrespective of whether the preferred method of our 70 said co-pending application is used or not.

Liquids, well adapted for the removal of the acetone are organic liquids such as benzene or its homologues, petroleum, or fractions of it;—certain acids such as diluted sulphuric acid;—and solutions of acid salts or neutral salts, for instance, a concentrated 75 solution of calcium chloride. Such solutions mix readily with the acetone but are entirely without effect upon the nitrocellulose and from all such liquids the acetone can be readily recovered for re-use by heating the liquid and driving off the acetone. It 80 will, of course, be obvious that in place of using acetone any of the well known homologues of acetone can be used, and we would state also that instead of using acetone or its homologues alone or in admixture with 85 each other, each of them may be mixed with other solvents of nitrocellulose such, for instance, as ethylalcohol.

Having now described our invention, what we claim as new and desire to secure 95 by Letters Patent, is:

1. The method of manufacturing clear unclouded products from nitrocellulose which consists in dissolving the nitrocellulose in a solvent made up in whole or in part of acetone or its homologues, imparting to the acetone collodion thus formed the desired 100 form and extracting the solvent by immersing the formed product in a liquid which is mixable with acetone and in which nitrocellulose is insoluble.

2. The method of manufacturing artificial silk filaments from nitrocellulose which consists in dissolving the nitrocellulose in a solvent made up in whole or in part of acetone or its homologues, forming the acetone collodion thus obtained into artificial silk filaments by forcing it through a spinnar-  
5 ette and extracting the solvent from the filaments by immersing them in a liquid which  
10 is mixable with acetone and in which nitrocellulose is insoluble.

3. The method of manufacturing artifi-

cial silk filaments from nitrocellulose which consists in dehydrating nitrocellulose hydrate, dissolving it in a solution made up 15 in whole or in part of dry acetone or its homologues, forming the acetone collodion into filaments by forcing it through spin-  
narettes and extracting the solvent from the filaments by immersing them in a liquid 20 which is mixable with acetone but in which nitrocellulose is not soluble.

EMILE BINDSCHEDLER.  
GEORGE JUER.